

1

3,825,497

## HYDRAULIC FLUIDS

Robert Alan Cameron Ker, London, England, assignor to  
 Castrol Limited, London, England  
 No Drawing. Continuation of abandoned application Ser.  
 No. 33,881, May 1, 1970. This application Apr. 28,  
 1972, Ser. No. 248,774  
 Int. Cl. C09k 3/00

U.S. CL. 252—79

5 Claims

## ABSTRACT OF THE DISCLOSURE

An improved hydraulic fluid is provided, which comprises a combination of two esters; one being a di (oxy-alkene) or di (polyoxyalkene) ester of a dibasic carboxylic acid, e.g. in amounts of 30% to 60% by weight; and the other being an ester of a diol, particularly a glycol, and a monobasic carboxylic acid, e.g. in amounts of 25% to 55% by weight.

This is a continuation of application Ser. No. 33,881, filed May 1, 1970 and now abandoned.

## BACKGROUND OF THE INVENTION

This invention relates to hydraulic fluids and is particularly, but not exclusively, concerned with liquids employed as the power transmitting medium in hydraulic brake systems for vehicles, for example, motor cars and aeroplanes.

British Patent Specification No. 1,083,324 describes and claims a hydraulic system containing, as the functional fluid, a hydraulic fluid having a kinematic viscosity at  $-40^{\circ}\text{C}$ . of not more than 5000 cs. and either consisting of, or comprising at least 50% by weight of, at least one ester having the general formula



where R is a straight or branched chain alkylene group which contains at least 2 carbon atoms, R<sup>1</sup> is an alkyl radical having from 1 to 4 carbon atoms or a phenyl radical, R<sup>2</sup> is ethylene, propylene or butylene and n is an integer of from 0 to 3. British Patent Specification No. 1,083,324 also describes and claims a hydraulic fluid having a kinematic viscosity at  $-40^{\circ}\text{C}$ . of not more than 5000 cs. and comprising at least 50% by weight of at least one ester having the general formula



where R is straight or branched chain alkylene group which contains at least 2 carbon atoms, R<sup>1</sup> is an alkyl radical having from 1 to 4 carbon atoms or a phenyl radical, R<sup>2</sup> is ethylene, propylene or butylene and n is an integer of from 0 to 3 together with a minor proportion of a polyoxyalkylene glycol or polyoxyalkylene glycol ether. Useful brake fluids have been formulated in accordance with that patent but it has not yet been found possible to formulate a fluid which conforms with all the most stringent specifications of various manufacturers of automobiles and hydraulic systems.

## SUMMARY

According to the present invention there is provided an improvement in and/or a modification of the hydraulic system claimed in claim 1 of British Patent Specification No. 1,083,324 which contains, as the functional fluid, a

2

fluid comprising a mixture of two esters A and B, ester A having the general formula:



wherein R<sup>3</sup> is a straight or branched chain alkylene radical or mixture of straight or branched chain alkylene radicals containing from 2 to 4 carbon atoms; R<sup>4</sup>, R<sup>5</sup>, R<sup>7</sup> and R<sup>8</sup> are the same or different and each is an ethylene or propylene radical; R<sup>6</sup> and R<sup>9</sup> are the same or different and each is a methyl or ethyl radical; and p, q, s and t are integers such that the total number of carbon atoms in R<sup>4</sup>, R<sup>5</sup>, R<sup>7</sup>, and R<sup>8</sup> is from 6 to 10 and such that if either s or t is zero the other is at least one and if either p or q is zero the other is at least one; and ester B having the general formula:



wherein R<sup>10</sup> and R<sup>11</sup> are the same or different and each is an ethylene or propylene radical; and l and m are integers such that the total number of carbon atoms in R<sup>10</sup> and R<sup>11</sup> is from 5 to 9.

## 25 PREFERRED EMBODIMENTS OF THE INVENTION

Preferably the total number of carbon atoms in R<sup>4</sup>, R<sup>5</sup>, R<sup>7</sup> and R<sup>8</sup> is from 7 to 9 and more preferably ester A has the general formula:



wherein R<sup>3</sup>, R<sup>6</sup> and R<sup>9</sup> have the same significance as hereinbefore described and wherein R<sup>6</sup> and R<sup>9</sup> are preferably methyl and R<sup>3</sup> is preferably derived from a mixture of adipic, glutaric and succinic acids. It is particularly preferred that this mixture of acids consists of 15% to 40% adipic, 40% to 60% glutaric and 15% to 35% succinic acid, the percentages being by weight.

Preferably the total number of carbon atoms in R<sup>10</sup> and R<sup>11</sup> is from 6 to 8, particularly 6. In a particularly preferred embodiment of the invention ester B is a tri-ethylene glycol dipropionate, dipropylene glycol dipropionate or a mixture of dipropionate esters derived from low cut co-condensates of ethylene and propylene oxides, e.g. diethylene oxa propylene glycols and dipropylene oxa ethylene glycols.

50 Preferably the acidity of ester B should not exceed 0.1 mgm. KOH/g.

The fluid may contain from 3% to 10%, by weight based on the weight of the fluid, of a polyoxyalkylene glycol or ether thereof, which preferably has the general formula:



wherein R<sup>12</sup> is an alkylene radical, or a mixture of alkylene radicals, containing from 2 to 4 carbon atoms, R<sup>13</sup> is a hydrogen atom or an alkyl group containing 1 to 3 carbon atoms and u is an integer from 2 to 4. Preferably R<sup>12</sup> is an ethylene radical, R<sup>13</sup> is an ethyl group and u is 3.

60 The fluid may also contain a minor amount, for example from 1% to 10%, preferably 2% to 5%, by weight, based on the weight of the fluid, of a reaction product of ammonia or an amine and an alkylene oxide or mixture of alkylene oxides, preferably ammonia and propylene oxide.

65 The fluid also may contain a lubricity additive such as glycol di basic acid polyesters, for example in an amount from 1% to 7%, preferably 3% to 5%, by weight, based on the weight of the fluid, or a complex

ester. In one embodiment of the invention the polyester is derived from one or more dibasic acids such as:

|              |               |   |
|--------------|---------------|---|
| sebacic acid | glutaric acid | 5 |
| azelaic acid | succinic acid |   |
| adipic acid  | phthalic acid |   |

and one or more diols selected from alkylene diols such as:

|                  |                      |    |
|------------------|----------------------|----|
| neopentyl glycol | ethylene glycol      | 10 |
| 1-4 butane diol  | 1,2 propylene glycol |    |
| 1-6 hexane diol  |                      |    |

and polyoxyalkylene glycols such as:

|                     |                       |    |
|---------------------|-----------------------|----|
| di ethylene glycol  | di propylene glycol   | 15 |
| tri ethylene glycol | tri propylene glycol. |    |

Preferably the lubricity additive has an acidity of less than 2.0 mgm. KOH/g. when determined by IP method 1.A. This can be achieved by using an excess of glycol or end stoping with a C<sub>1</sub>-C<sub>4</sub> alkanol during its preparation. The molecular weight of the polyester or complex ester is preferably from 500 to 3,000, more preferably from 600 to 2,000.

The fluid of the present invention may also contain known corrosion inhibitors and additives to maintain the pH above 7.0, for example bis(3,4-epoxy-6-methyl-cyclohexylmethyl)adipate.

The fluid preferably contains 30% to 60%, more preferably 35% to 50%, by weight of ester A and 25% to 55%, more preferably 30% to 50%, most preferably 35% to 45%, of ester B, the percentages being by weight based on the weight of the fluid.

The present invention also provides the hydraulic fluids which comprise a mixture of the two esters A and B, as hereinbefore described. The present invention further provides a method of operating a hydraulic system, which method comprises introducing into the hydraulic system a hydraulic fluid comprising a mixture of the two esters A and B, as hereinbefore described and transmitting power by applying pressure to the hydraulic fluid.

The invention will now be illustrated with reference to the following examples, in which all parts are by weight.

#### EXAMPLE 1

|                                      |    |
|--------------------------------------|----|
| Parts                                | 45 |
| Ester A <sub>1</sub>                 | 60 |
| Triethylethylene glycol dipropionate | 40 |

Ester A<sub>1</sub> was an ester of diethylene glycol monomethyl ether and a mixture of adipic acid (30.2%), glutaric acid (49.2%) and succinic acid (20.6%).

#### EXAMPLE 2

|                                    |    |
|------------------------------------|----|
| Parts                              | 55 |
| Ester A <sub>1</sub>               | 60 |
| Triethylene glycol dipropionate    | 30 |
| Triethylene glycol monoethyl ether | 10 |

#### EXAMPLE 3

|                                    |    |
|------------------------------------|----|
| Parts                              | 60 |
| Ester A <sub>1</sub>               | 70 |
| Diethylene glycol dipropionate     | 20 |
| Triethylene glycol monoethyl ether | 10 |

#### EXAMPLE 4

|                                                                                       |    |
|---------------------------------------------------------------------------------------|----|
| Parts                                                                                 | 65 |
| Ester A <sub>2</sub>                                                                  | 55 |
| Ester B <sub>2</sub>                                                                  | 35 |
| Triethylene glycol monoethyl ether                                                    | 7  |
| Amine A [a condensation product of propylene oxide (5.5 moles) with ammonia (1 mole)] | 3  |

Ester A<sub>2</sub> was a similar ester to Ester A<sub>1</sub> except that the proportions of adipic, glutaric and succinic acids were 16.6%, 57.8% and 25.6% respectively.

Ester B<sub>2</sub> was a co-condensation product of 2 moles ethylene oxide with one mole of propylene glycol ester- 75

fied with propionic acid and had a viscosity of 597 cs. at -40° F. and an SAE boiling point of 530° F.

The blends of Examples 1 to 4 were all found to be adequate brake fluids.

#### EXAMPLE 5

|                                 |      |
|---------------------------------|------|
| Parts                           |      |
| Ester A <sub>1</sub>            | 55   |
| Triethylene glycol dipropionate | 35   |
| Ethyl triglycol                 | 7    |
| Amine A                         | 3    |
| Dibutylamine                    | 0.1  |
| Benzotriazole                   | 0.1  |
| Triphenyl phosphite             | 0.15 |

This blend passed all the requirements of the SAE J1703 specification.

#### EXAMPLE 6

|                                    |      |
|------------------------------------|------|
| Parts                              |      |
| Ester A <sub>1</sub>               | 42   |
| Triethylene glycol dipropionate    | 45   |
| Triethylene glycol monoethyl ether | 7    |
| Amine A                            | 3    |
| Lubricity additive                 | 3    |
| Dibutylamine                       | 0.1  |
| Benzotriazole                      | 0.1  |
| Triphenyl phosphite                | 0.15 |

The lubricity additive was a complex ester sold under the trade name Reoplex 641, which had a molecular weight of 712 and was derived from neopentyl glycol and a mixture of sebacic, azelaic and adipic acids, the proportions of the acids in the mixture being determined, by analysis, as 53%, 5% and 38% respectively.

This blend passed the requirements of the SAE J1703 specification and specifications laid down by the brake manufacturers and automobile manufacturers.

#### EXAMPLE 7

|                                         |      |
|-----------------------------------------|------|
| Parts                                   |      |
| Ester A <sub>1</sub>                    | 39   |
| TEGDP (triethylene glycol dipropionate) | 45   |
| Triethylene glycol monoethyl ether      | 5    |
| Triethylene glycol monomethyl ether     | 5    |
| Amine A                                 | 3    |
| Reoplex 641                             | 3    |
| Dibutylamine                            | 0.05 |
| Benzotriazole                           | 0.05 |
| Agerite resin D                         | 0.05 |
| Armeen 12D                              | 0.1  |
| Triphenyl phosphite                     | 0.15 |

Agerite resin D is a commercially available polymerised trimethyl dihydro quinoline resin and Armeen 12D is a commercially available saturated straight chain primary amine wherein the straight chain is 95% C<sub>12</sub>, 3.5% C<sub>14</sub> and 1.5% C<sub>10</sub>.

#### EXAMPLES 8 TO 14

The blends of these examples were the same as Example 7, except in that the ester A<sub>1</sub> and triethylene glycol dipropionate were replaced by other esters as follows:

##### Example 8

30 parts DEDGS [the ester of diethylene glycol monomethyl ether and succinic acid]; 54 parts triethylene glycol dipropionate

##### Example 9

30 parts DMDGS [the ester of diethylene glycol monomethyl ether and succinic acid]; 54 parts triethylene glycol dipropionate

##### Example 10

55 parts DEDGA [the ester of diethylene glycol monomethyl ether and adipic acid]; 29 parts triethylene glycol dipropionate

## 5

## Example 11

54 parts DMDGA [the ester of diethylene glycol mono-methyl ether and adipic acid]; 30 parts triethylene glycol dipropionate

## Example 12

45 parts DEDGN [the ester of diethylene glycol mono-ethyl ether and a mixture of adipic acid (30.2%), glutaric acid (49.2%) and succinic acid (20.6%)]; 39 parts triethylene glycol dipropionate

## Example 13

45 parts DEDGG [the ester of diethylene glycol mono-ethyl ether and glutaric acid]; 39 parts triethylene glycol dipropionate

## Example 14

54 parts DMDGG [the ester of diethylene glycol mono-methyl ether and glutaric acid]; 30 parts triethylene glycol dipropionate.

The rubber swell characteristics of the blends of Examples 7 to 14 were determined by immersing a SBR (styrene-butadiene rubber) cup in the blends for 3 days at 120° C. and measuring the change in diameter of the cup. Further rubber swell characteristics determinations were made by the Archimedean principle described in British Patent Specification No. 1,083,324 by immersing samples of a synthetic rubber (designated G9) and a natural rubber (designated R32) in the blends. The results obtained, and other properties, are compared in the following Table with the results obtained, and the properties of, the esters (unblended) forming the major constituents of the blends.

wherein  $R^3$  is a straight chain alkylene radical containing from 2 to 4 carbon atoms and  $R^6$  and  $R^9$  are the same or different and each is a member selected from the group consisting of a methyl radical and an ethyl radical; and ester B being present in an amount of from 25% to 50% by weight and consisting of triethylene glycol dipropionate.

2. The fluid of claim 1 wherein ester A is a mixture of esters derived from a mixture of from 15% to 40% by weight adipic acid, 40% to 60% by weight glutaric acid and 15% to 35% succinic acid.

3. The fluid of claim 1 which also contains from 3% to 10% by weight, based on the weight of the fluid, of a polyoxyalkylene glycol or ether thereof having the formula:



wherein  $R^{12}$  is a member selected from the group consisting of alkylene radicals containing from 2 to 4 carbon atoms and mixtures thereof,  $R^{13}$  is a member selected from the group consisting of a hydrogen atom and an alkyl group containing from 1 to 3 carbon atoms and  $u$  is an integer of from 2 to 4.

4. The fluid of claim 3 wherein  $R^{12}$  is an ethylene radical,  $R^{13}$  is an ethyl group and  $u$  is 3.

5. The fluid of claim 1 which also contains, as a lubricity additive, from 1% to 7% by weight, based on the weight of the fluid of a polyester having a molecular weight of from 500 to 3,000 and derived from a dibasic acid selected from the group consisting of sebacic acid, azelaiic acid, adipic acid, glutaric acid, succinic acid, phthalic acid and mixtures thereof and a diol selected from the group consisting of neopentyl glycol, 1-4 butane diol, 1-6 hexane diol, ethylene glycol, 1,2-propylene glycol, di ethylene glycol, tri ethylene glycol, di propylene glycol and tri propylene glycol.

|                      | Viscosity<br>at -40° C.<br>(cs.) | Chemical<br>stability<br>°C.* | B.P.<br>(°F.) | SBR cup<br>3 days at<br>120° C.,<br>mm. | Shore<br>hardness,**<br>degrees | G9 rubber, percent |        | R32 rubber, percent |        |
|----------------------|----------------------------------|-------------------------------|---------------|-----------------------------------------|---------------------------------|--------------------|--------|---------------------|--------|
|                      |                                  |                               |               |                                         |                                 | 3 days             | 7 days | 3 days              | 7 days |
| TE GDP               | 670                              | +1                            | 560           | +1.91                                   | -13                             | 30.8               | 31.6   | 7.3                 | 7.4    |
| Example 7            | 1,620                            | -1                            | 575           | +1.03                                   | -4                              | 12.9               | 14.6   | 4.0                 | 3.8    |
| Ester A <sup>1</sup> | 3,790                            | +1                            |               |                                         |                                 | 6.9                | 8.2    |                     |        |
| Example 8            | 1,732                            | -1                            | 553           | +1.55                                   | -12                             | 20.8               | 20.8   | 4.9                 | 6.3    |
| DED GS               | 11,664                           | (**)                          |               |                                         |                                 | 18.1               |        | 3.5                 |        |
| Example 9            | 1,852-1,862                      | -0.5                          | 538           | +1.24                                   | -5                              | 16.7               | 16.5   | 4.0                 | 5.2    |
| DED GS               | 10,106                           | -1                            |               |                                         |                                 | 7.5                |        | 1.1                 |        |
| Example 10           | 1,773                            | +1                            | 536           | +1.44                                   | -6                              | 18.6               | 20.2   | 4.8                 | 5.7    |
| DE GDA               |                                  | +2                            |               |                                         |                                 | 14.1               |        | 5.5                 |        |
| Example 11           | 1,748                            | (**)                          | 545           | 9.15                                    | -2                              | 13.9               | 14.5   | 2.8                 | 3.3    |
| DMD GA               | 2,599                            | +3                            |               |                                         |                                 | 31.2               |        | 0.6                 |        |
| Example 12           | 1,756                            | -2                            | 551           | +1.46                                   | -9                              | 22.2               | 20.9   | 8.1                 | 4.9    |
| DED GN               |                                  | +1                            |               |                                         |                                 | 17.6               |        | 6.2                 |        |
| Example 13           | 1,806                            | +2                            | 556           | +1.61                                   | -9                              | 19.7               | 21.0   | 5.0                 | 4.8    |
| DED GG               | 3,305                            | -1                            |               |                                         |                                 | 19.7               | 17.2   | 2.4                 | 2.4    |
| Example 14           | 1,808                            | -2                            |               | +0.91                                   | -7                              | 11.0               | 11.6   | 2.9                 | 3.5    |
| DMD GG               | 2,526                            | -2                            |               |                                         |                                 |                    |        |                     |        |

\*According to S.A.E. J1703 Specification.

\*\*Shore Hardness of SBR cup after immersion as compared with Shore Hardness before immersion.

\*\*\*No change.

In general the results obtained in these rubber swell characteristics determinations were at least as good as, and in many cases substantially better than, the characteristics which would have been expected from a theoretical calculation thereon on the basis of the rubber swell characteristics of the individual constituents of the blends.

The fluids of the present invention also have the advantage of very low hygroscopicity and are similar in this characteristic to the fluids described in British Patent Specification No. 1,083,324.

I claim:

1. A hydraulic fluid consisting essentially of a mixture of two esters A and B, ester A being present in an amount of from 30% to 60% by weight and consisting of at least one compound of the formula:



$R_3$ !



## References Cited

## UNITED STATES PATENTS

- 60 2,542,785 2/1951 Walker ----- 252-79  
3,003,968 10/1961 Bruce et al. ----- 252-79  
3,029,204 4/1962 Matuszak et al. ----- 252-396 X  
3,056,745 10/1962 Morschel et al. ----- 252-79 X  
3,464,925 9/1969 Benoit et al. ----- 252-77  
65 3,623,987 11/1971 Ker et al. ----- 252-79  
3,637,507 1/1972 Gentit ----- 252-79

LEON D. ROSDOL, Primary Examiner

H. A. PITLICK, Assistant Examiner

U.S. Cl. X.R.

252-396